

Feb. 11, 1941.

C. V. FOERSTER, JR., ET AL 2,231,760

## METHOD OF REDUCING IRON ORES AND THE LIKE

Filed July 12, 1939



Fig. 3



Fig. 1



Fig. 2  
INVENTOR

CHARLES V. FOERSTER, JR.  
HOWARD L. GRISWOLD  
ARTHUR T. CAPE

BY

ARTHUR T. CAPE  
Horace B. Fay  
ATTORNEY.

## UNITED STATES PATENT OFFICE

2,231,760

METHOD OF REDUCING IRON ORES AND  
THE LIKECharles V. Foerster, Jr., Howard L. Griswold, and  
Arthur T. Cape, Santa Cruz, Calif.

Application July 12, 1939, Serial No. 234,076

3 Claims. (Cl. 75—34)

This invention relates, as indicated, to a method of reducing iron ores and the like.

A primary object of the invention is to provide a method whereby iron ores may be reduced to sponge iron in an economical and highly efficient manner.

Another object of the invention is to provide a method of producing sponge iron of an excellent grade, such as is desirable for making pressed metal products.

Other objects and advantages of the invention will be apparent during the course of the following description.

In the accompanying drawing, forming a part of this specification, and in which like numerals are employed to designate like parts throughout the same.

Fig. 1 is a fragmentary view, showing apparatus which may be employed for practicing the present invention;

Fig. 2 is a vertical cross-sectional view, on an enlarged scale, showing the reducing tower; and

Fig. 3 is a transverse cross-sectional view, taken on the line 3—3 of Fig. 2.

Referring more particularly to the drawing, A designates generally a furnace formed of a suitable refractory material and comprising a reducing gas inlet portion 1, a portion 2 for supplying heat to the reducing tower, and a tower portion 3.

Disposed vertically within the tower portion 3 of the furnace is a metallic tower B, preferably formed of a heat and corrosion-resistant alloy steel and of generally cylindrical form, and consisting of a lower section 4 and an upper section 5, separated from each other, as by an annular plate 6, which is desirably welded or otherwise secured to either the upper end of the lower section or lower end of the upper section. The tower sections thus provide a lower chamber C and an upper chamber D.

Secured, as by welding, to the outer surface of the section 4 adjacent its upper end is a collar 7, which extends upwardly sufficiently to overlap the outer surface of the section 5 adjacent its lower end. The collar 7 is thus effective to not only seal the joint between the tower sections, but enable the upper section to be centralized with respect to the lower section, when assembling the tower sections.

A substantially gas-tight seal between the tower sections is effected by securing to the collar 7 a sleeve 8, the upper portion of which is spaced from the tower section 5, and filling the annular

space thus formed with a suitable refractory cement 9.

The tower section 4 rests on an annular plate 10 mounted on the base of the tower portion of the furnace, and a collar 11, which may be secured to the plate 10 provides a seal at this point and serves to facilitate the central positioning of the tower section 4.

Mounted within the lower end of the tower section 4 is a hopper 12 which communicates 10 with a conduit 13, within the upper end of which is secured a nozzle 14 having a central vertical passageway 15 and a plurality of radially extending openings 16 communicating the interior of the conduit 13 with such passageway 15. 15 The upper surface of the nozzle 14 is in effect a continuation of the hopper surface, thereby facilitating the discharge of the reduction products, as will be presently described.

A conduit 17, which serves a purpose to be presently described, is in communication with the conduit 13, and the conduit 13, in turn is connected as by means of a discharge pipe 18 with a sponge cooler 19. A plug 20 is movable vertically within the pipe 18 and conduit 13 and 25 is adapted, at times, to close the passageway 15 in the nozzle 14.

A hopper 21, similar to the hopper 12, is mounted within the lower end of the tower section 5 and is adapted to discharge the contents 30 of said tower section into the tower section 4 through a nozzle 22, which is similar in all respects to the nozzle 14, that is to say, it has a vertically extending passageway 23 and a plurality of radially extending openings 24, which 35 communicate the interior of the tower section 5 with such passageway 23.

Each of the tower sections 4 and 5 is provided with a multiplicity of circumferentially spaced radially extending reinforcing fins or ribs 25, 40 which are also effective to increase the heat-retentivity of such tower sections.

Secured, as by hold-down rods 26, to brackets 27 within the upper end of the tower section 5, is an exhaust gas header 28 having an opening 45 29 therein for charging the ores or like products to be reduced into the chamber D. A reducing gas exhaust stack 30 extends upwardly, in an inclined direction from the header 28, and has a damper 31 mounted therein. A number of 50 circumferentially spaced poke-hole openings 32 are provided in the base flange 33 of the header 28, and a gas-tight seal is provided between the tower section 5 and the flange 33 by filling the annular space between a ring 34, secured to the 55

base flange 33, and the upper end of the tower section 5, with cement packing 35.

Means are also provided, in the form of a burner nozzle 36, for supplying heat to the space 5 which surrounds the tower sections 4 and 5 for heating such sections, the exhaust gases being discharged through a stack 37.

Thermo-couple wells 38 and 39 are provided for respectively determining the temperatures 10 within and without the reducing tower sections, and slotted tubes 40 and 41 are also provided for extraction of analysis samples of the gases within these tower sections. Sight tubes 42 are also provided for observing conditions within the 15 tower section 4.

The apparatus which has been described is particularly adapted for reducing ores in a relatively fine state of subdivision, such for example, as certain sands, massive ores which have 20 been crushed and sized, as well as iron oxide obtained from various chemical processes.

For the purpose of reducing these ores and/or oxides, a reducing gas is employed, such gas being 25 preferably one consisting of a mixture of carbon monoxide, hydrogen and nitrogen, and containing a minimum of carbon dioxide and water vapor. Such a gas is produced, for example, by the method disclosed in the United States Re-issue Patent No. 19,770 to William D. Brown. 30 The hot gases, produced in accordance with the aforesaid patent, are introduced into the apparatus through the conduit 17 and pass upwardly into the chamber C through the conduit 13 and nozzle 14 and into the chamber D through the 35 nozzle 22. At the same time, the ore or oxide which is to be reduced, is introduced into the chamber D through the opening 29, and by suitable adjustment of the gas flow, the ore or oxide is maintained in the chamber D, the velocity of 40 the gases in the passageway 23 of the nozzle 22 being sufficient to overcome any tendency of the ore in the chamber D to pass downwardly through such passageway. The velocity of the gases which pass into the chamber D is sufficient to 45 maintain the ore in a relatively violent state of agitation, so that the gases are thoroughly intermingled with the ore and the ore is partially reduced in the chamber D.

With the ore thus partially reduced, the flow of 50 gases into the chamber D is decreased or entirely stopped, permitting the partially reduced ore to fall through the passageway 23 of the nozzle 22 and into the chamber C, the plug 28 having first been elevated to close the lower end of the passageway 15 in the nozzle 14, to thereby prevent any of the partially reduced ore from falling into the conduit 13. The flow of gases in the chamber C is then resumed, the gases entering the chamber through the radial openings 16 and passageway 15 in the nozzle 14. The velocity of 55 these gases, in their passage through the relatively small passageway 15, is sufficient to overcome any tendency of the partially reduced ore in the chamber C to pass downwardly through such passageway, it being understood that as soon as the flow of gases has been resumed, the plug 28 is lowered. The velocity of the hot gases which pass into the chamber C is sufficient to maintain the partially reduced ore in a violent state of 60 agitation, so that the gases are thoroughly intermingled with such ore, and the reduction of the ore is completed.

When the flow of gases into the chamber C has 65 been resumed, and a sufficient time interval has 70 elapsed for such gases to pass upwardly into the

chamber D, a second charge or batch of ore is introduced into the chamber D.

When the ore in the chamber C has been completely reduced, the flow of gases is decreased or stopped, permitting the sponge iron to fall 5 through the passageway 15, through conduit 13 and pipe 18 into a cooler 19. At the same time the partially reduced ore in the chamber D falls into the chamber C.

The burner 36 supplies sufficient heat to the 10 tower sections 4 and 5 to compensate for radiation losses, so that the heat necessary for the reducing reactions is supplied primarily by the reducing gases themselves. In other words, the heat is supplied under most efficient conditions. 15 Moreover, the gas-ore contact is ideal, and no mechanical parts are essential to the satisfactory operation of the apparatus.

The reducing reactions are primarily between the iron oxide and the carbon monoxide and 20 hydrogen.

The method thus embodies the counter-current principle of operation, but is intermittent to the extent that the ore is not falling continuously but is maintained in each of the chambers for a period 25 of time sufficient to produce the degree of reduction desired in such chamber. As the gases rise, they become increasingly cooler, of course, so that the minimum degree of reduction occurs in the upper or cooler portion of the tower, and the 30 maximum degree of reduction in the lower or hotter portion of the tower.

It will be understood that the apparatus need not necessarily be confined to the use of two superposed tower sections, but that as many sections and chambers as may be required to accomplish the desired reduction may be employed, depending on the nature of the ore, the state of subdivision thereof, and other factors well known in the art to which this invention relates. Moreover, it is not essential that the tower sections be cylindrical or that they be of uniform cross-sectional area throughout.

It is to be understood that the form of our invention, herewith shown and described, is to be 45 taken as a preferred example of the same, and that various changes in the shape, size and arrangement of parts may be resorted to, without departing from the spirit of our invention, or the scope of the subjoined claims.

Having thus described our invention, we claim:

1. In a method of reducing iron ores and the like in a vertical tower having vertically-spaced ore passage points of restricted cross-sectional area, the steps which comprise flowing the ore downwardly in said tower and flowing hot reducing gases upwardly through the tower in counter-current relation to the flow of ore, the velocity of the gases through said points of restricted cross-sectional area being sufficient to overcome 60 any tendency of the ore passing downwardly through said points, and intermittently decreasing or stopping the flow of gases to permit the reduced or partially reduced ore to flow through said points of restricted cross-sectional area. 65

2. In a method of reducing iron ores and the like in a vertical tower having a point of restricted cross-sectional area, the steps which comprise flowing the ore downwardly in said tower and flowing hot reducing gases upwardly through 70 said point of restricted area and into said tower, the velocity of said gases at said point being sufficient to prevent the ore from flowing downwardly through said point of restricted area and the velocity of the gases which pass into said 75

5 tower above said point being sufficient to maintain the ore in a relatively violent state of agitation, so that the gases are thoroughly intermingled with the ore, and then decreasing the flow of gases sufficiently to permit the ore to fall through said point of restricted area.

10 3. In a method of reducing iron ores and the like in a vertical tower having at least two vertically-spaced reaction chambers and points of smaller cross-sectional area than said chambers below said chambers, the steps which comprise 15 flowing the ore downwardly in said tower and into the uppermost chamber, flowing hot reducing gases upwardly through the uppermost of said points and into said uppermost chamber, the velocity of the gases passing through said upper-

most point being sufficient to prevent the ores from flowing downwardly through said uppermost point, reducing the gas pressure to permit the partially reduced ore to flow through said upper point, flowing hot reducing gases upwardly 5 through the lower of said points and into the lower chamber, the velocity of the gases passing through said lower point being sufficient to prevent the partially reduced ore from flowing through said lower point, and then reducing the 10 gas pressure to permit the ore in said lower chamber to flow through said point.

CHARLES V. FOERSTER, JR.

HOWARD L. GRISWOLD.

15

ARTHUR T. CAPE.